

## UNITED STATES PATENT OFFICE

2,176,884

PROCESS FOR PRODUCING AN IMPROVED  
LUBRICATING OIL

John G. Butz, Philadelphia, and Leonard N. Leum, Lansdowne, Pa., assignors to The Atlantic Refining Company, Philadelphia, Pa., a corporation of Pennsylvania

No Drawing. Application September 23, 1937,  
Serial No. 165,312

## 7 Claims. (Cl. 196—147)

The present invention relates to the treatment of lubricating oils, and relates more particularly to the improvement of properties such as color, viscosity-temperature susceptibility and film strength of lubricating oils.

In accordance with the present invention, lubricating oil stocks, particularly those derived from petroleum distillates or residuums, are treated with phosphorus sulfo-chloride,  $\text{PSCl}_3$ , preferably in the presence of an agent such as  $\text{AlCl}_3$ ,  $\text{FeCl}_3$ ,  $\text{ZnCl}_2$ ,  $\text{SnCl}_4$  or  $\text{BF}_3$ . Such treatments may be carried on at atmospheric or higher temperatures, and preferably at temperatures of from about  $100^\circ \text{C}$ . to about  $200^\circ \text{C}$ . The quantity of  $\text{PSCl}_3$ , and of an agent such as, for example,  $\text{AlCl}_3$ , employed, may each be of the order of from about 1% to 10% or more, by weight, based upon the quantity of oil treated. For example, the ratio of  $\text{PSCl}_3$  to  $\text{AlCl}_3$  to an oil may be 2:2:100;

20

and the admixture heated, with agitation, to about  $100^\circ \text{C}$ . for a period of about 5 hours. The treated oil was then cooled and separated from any insoluble reaction products, i. e., sludge, and the oil was thereafter washed with water and 10% sodium hydroxide solution and dried by air blowing. The properties of the initial oil stock and the oils treated with varying amounts of reagents, are shown in the following table. The viscosity index was determined in accordance with the method of Dean & Davis (Chemical & Metallurgical Engineering, vol. 36, page 618), while the film strength was determined in an Almen extreme pressure lubricant testing machine operated at 200 R. P. M. The pressures indicated are pounds per sq. in. projected bearing area sustained before failure of the test bearing.

20

Table I

| Reagents weight, percent | Color           |                 | Viscosity (S. U.) |         | Viscosity index | Film strength, lbs./sq. in. | Yield   |
|--------------------------|-----------------|-----------------|-------------------|---------|-----------------|-----------------------------|---------|
|                          | $\text{PSCl}_3$ | $\text{AlCl}_3$ | N. P. A.          | O. D.   |                 |                             |         |
| 0.0                      | 0.0             | >8              | 179               | Seconds | 647             | 71.6                        | 98      |
| 8.1                      | 7.7             | 1.5             | 4                 | 451     | 62.7            | 105                         | 22,000+ |
| 4.5                      | 7.7             | 1.5             | 4                 | 431     | 61.7            | 106                         | 21,000  |
| 4.5                      | 3.8             | 2.0             | 8                 | 544     | 67.9            | 103                         | 19,000  |
| 2.0                      | 7.7             | 1.0             | 1                 | 452     | 63.2            | 107                         | 14,000  |
| 0.0                      | 7.7             | 1.25            | 2                 | 463     | 63.4            | 106                         | 7,000   |
| 8.1                      | 0.0             | 6.25            | 149               | 653     | 72.4            | 99                          | 12,000  |

20

25

2:5:100; 5:4:100; 5:8:100; 8:8:100; or 10:10:100, depending upon the nature of the oil to be treated and upon the qualities desired of the lubricant. In general, the higher the percentage of  $\text{PSCl}_3$  employed, the greater will be the film strength or load-bearing capacity of the treated oil, and the higher the percentage of an agent such as  $\text{AlCl}_3$ , the greater will be the improvement in viscosity-temperature susceptibility or viscosity index. While we prefer to employ a combination of  $\text{PSCl}_3$  and an active metallic halide such as  $\text{AlCl}_3$ , we may simply employ  $\text{PSCl}_3$ , in which case an improvement in film strength is obtained, with little change in color or viscosity index. However, by utilizing  $\text{PSCl}_3$  and an active metallic halide, higher film strength may be obtained than with  $\text{PSCl}_3$  alone, and, in addition, the color and viscosity index are markedly improved.

Our invention may be further illustrated by the following examples, in which a lubricating oil distillate was admixed with  $\text{PSCl}_3$  and  $\text{AlCl}_3$ ,

It will be seen from the above examples, that while treatment with  $\text{PSCl}_3$  alone improves the film strength of the oil, and that treatment with  $\text{AlCl}_3$  alone improves the color and viscosity index of the oil, the combination of  $\text{PSCl}_3$  and  $\text{AlCl}_3$  produces not only color and viscosity index improvement but a marked increase in film strength over that obtained with  $\text{PSCl}_3$  alone.

In the following examples, in which our process is applied to a variety of oil stocks, the treatment consists essentially in mixing 100 parts by weight of oil with 5 parts by weight of  $\text{PSCl}_3$  and 6.2 parts by weight of  $\text{AlCl}_3$ , heating the mixture, with agitation, to about  $100^\circ \text{C}$ . for about 5 hours, cooling the mixture and separating any insoluble reaction products therefrom, washing the treated oil with water and with 10% sodium hydroxide solution, and finally air drying the treated oil. The properties of the untreated oil stocks and the products resulting from the treatment thereof are shown in Table II.

25

40

45

50

55

Table II

| Oil stock                                                          | Color<br>O. D. | Viscosity (S. U.) |         | Viscosity<br>index | Film<br>strength | Yield    | 5  |
|--------------------------------------------------------------------|----------------|-------------------|---------|--------------------|------------------|----------|----|
|                                                                    |                | 100° F.           | 210° F. |                    |                  |          |    |
| 5 Solvent extracted S. A. E. 30 motor oil (untreated)              | 13.5           | Seconds           | Seconds | 86                 | 4,000            | Per cent |    |
| Same, treated with $\text{PSCl}_3$ and $\text{AlCl}_3$             | Colorless      | 379               | 55.2    | 98                 | 22,000+          | 89       |    |
| 10 Solvent extract fraction from S. A. E. 30 motor oil (untreated) | 670            | 491               | 51.2    | -16                | 3,000            |          | 10 |
| Same, treated with $\text{PSCl}_3$ and $\text{AlCl}_3$             | 56             | 314               | 49.0    | 49                 | 22,000+          | 60       |    |
| 15 Solvent extracted residuum from East Texas crude (untreated)    | 317            | 2,547             | 144.0   | 88                 | 4,000            |          |    |
| Same, treated with $\text{PSCl}_3$ and $\text{AlCl}_3$             | 65             | 1,555             | 108.2   | 88                 | 22,000+          | 85       |    |
| Lubricating oil distillate from East Texas crude (untreated)       | 290            | 942               | 68.5    | 33                 | 3,000            |          |    |
| Same, treated with $\text{PSCl}_3$ and $\text{AlCl}_3$             | 29             | 516               | 58.5    | 64                 | 22,000+          | 75       |    |
| 15 Residuum from East Texas crude (untreated)                      | 10,650         | 5,368             | 177.2   | 55                 | 9,000            |          |    |
| Same, treated with $\text{PSCl}_3$ and $\text{AlCl}_3$             | 292            | 3,065             | 132.6   | 59                 | 22,000+          | 80       |    |

In the foregoing description and examples we have shown the application of our process in the treatment of hydrocarbon lubricating oils. Such treated oils may be employed, per se, as lubricants, or may be admixed in any desired proportion with other hydrocarbon oils, fatty oils, sulfurized or chlorinated oils, esters, metal soaps, greases and the like. However, in accordance with our invention we may also treat a mixture of hydrocarbon oil and a fatty oil, for example, lard oil, castor oil, sperm oil, cotton seed oil or the like, when it is desirable to provide a lubricant containing fatty oil compounds. Or, alternatively, we may treat a fatty oil with  $\text{PSCl}_3$ , or  $\text{PSCl}_3$  and an active metallic halide such as  $\text{AlCl}_3$ , and thereafter add such treated fatty oil to a hydrocarbon lubricating oil which may have been subjected to our treatment hereinbefore described.

Our process may be applied to oils from practically any source, for example, untreated petroleum distillates or residuums; acid treated oils; clay treated oils; solvent treated oils; oils produced by hydrogenation; oils produced by cracking; and oils produced by various synthetic or polymerization methods.

What we claim is:

45 1. A process for producing an improved lubricating oil which comprises treating hydrocarbon oil containing lubricating oil components with a reagent comprising  $\text{PSCl}_3$  at a temperature of from substantially atmospheric to about 200° C., and separating from the treated oil any insoluble reaction products resulting from such treatment.

2. A process for producing an improved lubricating oil which comprises treating hydrocarbon oil containing lubricating oil components with  $\text{PSCl}_3$  and an active metallic halide from the group consisting of  $\text{AlCl}_3$ ,  $\text{FeCl}_3$ ,  $\text{ZnCl}_2$ ,  $\text{SnCl}_4$

and  $\text{BF}_3$  at a temperature of from substantially atmospheric to about 200° C., and separating from the treated oil any insoluble reaction products resulting from such treatment.

3. A process for producing an improved lubricating oil which comprises treating hydrocarbon oil containing lubricating oil components with  $\text{PSCl}_3$  and  $\text{AlCl}_3$  at a temperature of from substantially atmospheric to about 200° C., and separating from the treated oil any insoluble reaction products resulting from such treatment.

4. A process for producing an improved lubricating oil which comprises treating hydrocarbon oil containing lubricating oil components with  $\text{PSCl}_3$  and  $\text{AlCl}_3$  at a temperature of from about 100° C. to about 200° C., and separating from the treated oil any insoluble reaction products resulting from such treatment.

5. A process for producing an improved lubricating oil which comprises treating hydrocarbon oil containing lubricating oil components with a mixture of about 1% to about 10% by weight of  $\text{PSCl}_3$  and about 1% to about 10% by weight of  $\text{AlCl}_3$  at a temperature of from substantially atmospheric to about 200° C., and freeing the treated oil of undesirable reaction products resulting from such treatment.

6. In a process for producing an improved lubricating oil, the step which comprises subjecting a lubricating oil to the action of a reagent comprising  $\text{PSCl}_3$  at a temperature of from substantially atmospheric to about 200° C.

7. In a process for producing an improved lubricating oil, the step which comprises subjecting a lubricating oil to the action of  $\text{PSCl}_3$  and  $\text{AlCl}_3$  at a temperature of from substantially atmospheric to about 200° C.

JOHN G. BUTZ.

LEONARD N. LEUM.